

June 28, 1938.

H. H. FONDA

2,121,909

TEXTILE FABRIC AND METHOD OF MAKING THE SAME

Filed Aug. 31, 1937

FIG. 1.



FIG. 2.



FIG. 4.



FIG. 3.



H. H. Fonda

Robt. Robb,  
By  
Attorneys

## UNITED STATES PATENT OFFICE

2,121,909

TEXTILE FABRIC AND METHOD OF MAKING  
THE SAMEHarold H. Fonda, Skaneateles, N. Y., assignor to  
Nye-Walt Company, Inc., Auburn, N. Y., a corporation of New York

Application August 31, 1937, Serial No. 161,866

14 Claims. (Cl. 139—391)

This invention appertains to a new and improved textile pile fabric and method of making the same, and more especially, to the manufacture of carpets or rugs having artistic figurative designs formed in relief on the face of the fabric. In a broad sense, the design may be said to be an embossed design which is attained by interweaving differentially twisted yarns in a predetermined pattern and subsequently treating the 5 yarns to release the twist of the harder twisted yarns, thereby causing certain of the pile tufts to rise above the others, or elongate and form a distinctive contrast against the field or background which is constituted by the other pile tufts. This 10 contrast is readily discernible irrespective of any difference in material composition of the yarns which form the pile tufts, or a contrast resulting from the employment of yarns of different colors. Of course, if desired, yarns of different composition 15 and/or colors may be employed to emphasize the embossed effect, but it is to be understood that this is not essential to the invention.

I am aware that mechanical shearing of the pile tufts to form figurative designs has been 20 practiced for many years, and the origin of such practice is generally attributed to the Chinese artisans of old. However, this old mechanical shearing method involved nothing more than the cutting of grooves or channels in the pile face of 25 the fabric in the form of figurative outlines, so that the pile areas outlined or bounded by these grooves or channels are merely separated from the other areas, and does not embrace the use of pile tufts of different heights within the respective 30 areas, as in the present invention.

Another old practice of forming figurative designs in pile fabrics is to employ yarns of different material composition such as a combination of yarns of animal and vegetable fibers which are 35 treated after weaving of the same in such manner that one set of yarns is destroyed or disintegrated, leaving the other yarns to form the pattern. This practice has never gone into extensive use, and is generally considered to be impractical. 40 I am also aware that the employment of differentially twisted yarns in pile fabrics, and the subsequent treatment of said yarns so as to cause certain of the pile tufts to sink down or mat below other pile tufts formed of other yarns having 45 a different twist, have been proposed to create frieze, pebbled or crepe effects, but this practice is likewise materially different from the method of producing my embossed pile fabric, as will hereinafter become more apparent.

50 One of the primary objects of my invention is

to produce embossed or relief designs in pile fabrics in a more practical and economical way than has been heretofore possible, and enabling the practical attainment of the same or a greater degree of beauty, as formerly obtained by the old mechanical hand-shearing method generally attributed to the Chinese artisans previously mentioned.

5 My invention attains the desired ends just referred to with a greater uniformity of surface 10 appearance of the fabric in the high and low pile areas, and affords a higher degree of density of the pile and greater coverage, thus contributing to a much longer and better wearing quality of both the low and high pile areas than in the 15 case of the old practices previously referred to.

Other objects and advantages of the invention will be hereinafter described, and the novel features thereof defined by the appended claims.

20 In the drawing:

Figure 1 is a fragmentary top plan view of a pile fabric embodying my invention, and illustrating the distinctive embossed effect in a typical figurative design, which has been shown merely as one example of the many artistic designs which 25 may be produced in the practice of my method;

Figure 2 is an enlarged fragmentary vertical sectional view, taken through the fabric of Figure 1 to illustrate the manner in which the pile tufts are bound in the fabric, and showing the 30 relationship of the long and short pile tufts which form the high and low pile areas on the surface of the fabric;

Figure 3 is a horizontal sectional view, taken approximately on the line 3—3 of Figure 2; and 35

Figure 4 is an enlarged fragmentary detail view in vertical section, illustrating the method of weaving the pile yarns in the fabric, the view representing one stage of the weaving operation prior to withdrawal of the pile wires and cutting 40 of the pile loops.

Like reference characters designate corresponding parts in the several figures of the drawing. The invention is especially applicable to a Wilton weave as obtained with a Jacquard 45 equipped loom, or an Axminster weave, or a Chenille weave, in each of which there is relatively little limitation in design and pattern. It is also applicable to other types of looms where more than one yarn can be handled simultaneously, as 50 in the case of a plain tap loom for producing two-tone effects. The resulting embossed effect which I am able to obtain must, of course, fall within the limitations of the pattern control of the loom or its mechanical arrangement for handling the 55

yarn. In the case of a Wilton weave, any portion of the rug can be made embossed, depending upon how the pattern is cut. If yarns of different colors are used, there will be one frame 5 for each colored yarn. The Jacquard picks up the yarn that the pattern calls for. In the case of an Axminster loom, the yarn would be selected in accordance with the embossed effect desired, at the time the yarn is placed in the setting frames, just as colors would be prepared in the ordinary way for the loom. In other words, the weaving operations in practicing my invention are carried out in the customary manner 10 of forming designs and patterns in pile fabrics 15 having an even surface, whereas the embossed effect is not produced in the actual weaving operation, but rather as a result of the subsequent treatment of the yarn.

In the drawing, I have shown my invention 20 embodied in a typical Wilton weave, wherein 1 designates the usual fine chain or binder warp, 2 the buried yarn and stuffer, and 3 the filling threads, which, together with the fine chain 1, bind the pile surface yarns, generally designated 25 4, to the backing fabric. The pile yarns 4 are woven in the usual manner over pile wires 5, as best seen in Figure 4, to form pile loops of substantially uniform height, and when the pile wires are withdrawn, the pile loops are cut and 30 cause the pile yarns to assume the form of tufts which are uniformly distributed over the face of the fabric. Thus, there is nothing novel in the weaving of the fabric itself.

To attain the embossed effects which characterize my invention, I employ differentially twisted pile yarns. As one specific example of the pile yarns employed in the fabric illustrated in the drawing, I take a single wool yarn having a twist of about forty-seven turns in ten inches, 35 and make up a three-ply yarn having a twist of about seventy-four turns in ten inches, the ply twist being in the opposite direction to the single twist. This three-ply yarn is employed for one of the sets of pile yarns which are embodied 40 in the fabric. This yarn is preferably treated before weaving the same into the fabric, in a water bath having a temperature of approximately 120 degrees F. for about twenty minutes, to temporarily set the ply twist. Where colored 45 yarns are employed, the yarn is preferably dyed in single before plying so as not to permanently set the ply twist. The bath to which the plied yarn is subjected after plying, as previously mentioned, should be maintained at a temperature 50 below that which would strip the yarn color, in the case of dyed yarns, and it is for this reason that I have selected a bath temperature of about 55 120 degrees F.

In contrast to the three-ply yarn above referred to, a second set of pile yarns is employed, which are preferably of two-ply construction, the single twist being the same as in the three-ply 60 yarn, and the two-ply twist being approximately twenty-eight turns in ten inches in the opposite 65 direction to the single twist. No bath treatment is required in the case of the two-ply yarn since the twist is not as great as in the harder twisted three-ply yarn.

Although two and three ply combination is 70 perhaps preferred, and is used in this instance as a means of explanation, other combinations of twist can be used to produce similar results.

The two yarns are placed in the loom in accordance with the design of the carpet or rug to 75 be produced, which, of course, is predetermined

just as in the case of any pattern where different colors are used. One of the advantages of my invention is that the yarns which are used to produce the long and short pile in the final fabric may be of the same kind and quality of fiber. 5 Wool yarn is preferred, but the invention is not limited thereto, and the yarns may be composed of the same or different blends of staple length fibers of a spinnable character. As previously mentioned, the fabric is woven in the same manner as any two-tone or figured fabric, and it comes off the loom with a relatively uniform pile height, just as in the case of ordinary pile carpet or rug fabrics. After weaving, the fabric is preferably sheared in the usual manner to insure that 10 all the pile tufts are of the same height, but this shearing operation is not absolutely necessary, and largely depends upon the quality desired. Ordinarily, the better quality fabrics are sheared 15 after weaving. At this stage, the fabric is next 20 given a wet treatment by washing the same in plain water, or with a suitable chemical solution, depending upon whether or not it is desired to impart a luster or sheen to the fabric. In the case of a chemical wash, the fabric is preferably 25 washed in a chlorinated lime solution for a period of approximately twenty minutes, and then in a formic acid solution for another period of approximately twenty minutes, the solutions being maintained at a temperature of approximately 30 ninety degrees Fahrenheit. Thereafter, the fabric should be rinsed in plain water for about five minutes, and when the fabric has been dried, it will have a beautiful luster or sheen.

The wet treatment in either plain water or the 35 chemical solutions referred to serves to partially release the twist of the harder twisted three-ply yarn, thereby causing the pile tufts formed by this set of yarns to elongate and rise above the pile tufts formed by the other set of two-ply 40 yarns, thereby creating high and low pile areas 4' and 4'', according to the pattern woven on the loom, as illustrated, for example, in Figure 1 of the drawing. This difference in the height of the pile is quite distinct, and gives the embossed effect in the final fabric. The wet treatment does not materially affect the lesser twisted two-ply 45 yarns, but does shrink the backing threads which are ordinarily composed of cotton. This shrinkage of the backing threads aids in securely binding 50 the pile yarns to the backing fabric.

A further effect of the wetting treatment on the pile yarns is to partially spread or open up the pile tufts, with the result that the pile surface becomes quite dense and is uniform throughout, affording an unusually high degree of coverage which materially contributes to the beauty and long wearing qualities of the fabric. After 55 the wet treatment, and when the fabric has been dried, it is again preferably sheared to give greater evenness to the high pile areas, but here again, the final shearing is a matter of choice, and depends upon the desired quality and surface appearance of the final fabric. The yarn in the high pile areas assumes a state of lesser ply twist 60 after the wet treatment, and is substantially the same in this respect as the yarn which forms the low pile areas, just as if the fabric were originally made with the same pile height over all. Of course, the bases or roots of the pile tufts which 65 form the high pile areas, will remain harder twisted than the bases or roots of the other pile tufts, due to the former being initially woven and bound in the backing fabric in a harder twisted state. The twist releasing result of the wetting 70

treatment is effective at least on the free ends of the tuft yarns, and substantially down to the tuft bases or roots.

From the foregoing, it will be readily understood that an effect compared to a two-tone effect can be created through the use of yarns of the same color in both the high and low pile areas. This is due to the shadows and highlights which result from the use of two pile heights.

10 The amount of increase in the pile height which results from the wet treatment largely depends upon the relative twist of the different yarns, and of course, I am not limited to the use of only two different pile heights, since more than 15 two different pile heights may be obtained through the employment of more than two sets of pile yarns, each having a different amount of twist.

15 The embossed effect emphasizes pattern designs where different colors are used, regardless of the form of the design, whether it be geometrical, floral, oriental, or otherwise. The construction has a distinct style appeal and is unusually serviceable, and does not readily loose its distinctiveness through wear or cleaning treatments, even where the cleaning treatment involves a washing operation. In this respect, my invention is a marked advantage over pebbled or frieze fabrics.

20 The references herein to two and three ply yarns and to the specific degrees of twist of the yarns in single or plied form, are not to be taken as fixed, but rather merely as one practical example of the construction. In other words, the 25 plied yarns may be composed of more than two or three single yarns and the ply twist may be varied more or less as desired, depending upon the quality and degree of differentiation between the high and low pile areas to be ultimately attained. It is important, however, that the twist of the 30 harder twisted yarns should not be so great as to cause the pile ends to curl over or mat down when subjected to a wetting treatment, and it is equally important that the twist be not permanently set prior to the wetting treatment.

35 While the specific details have been herein shown and described, the invention is not confined thereto, as changes and alterations may be made without departing from the spirit thereof as defined by the appended claims.

40 Having thus described my invention, what I claim as new and desire to secure by Letters Patent is—

1. The method of producing embossed or relief designs in pile fabrics, which comprises weaving twisted pile yarns composed of staple length fibers and having different degrees of twist, according to a predetermined pattern, to initially provide a pile surface composed of tufts of substantially uniform height, and thereafter subjecting said pile yarns to a wetting treatment whereby to partially release the twist of the harder twisted yarns so as to cause the pile tufts formed by these yarns to elongate and rise above the pile tufts formed by the other lesser twisted 45 yarns which are substantially unaffected by the wetting treatment.

50 2. The method of producing embossed or relief designs in pile fabrics, which comprises weaving a plurality of sets of multi-ply pile yarns, the 55 yarns of each set having a different degree of twist, according to a predetermined pattern, to initially provide a pile surface composed of tufts of substantially uniform height, the component strands of each set of pile yarns being individually twisted in one direction and plied by twisting

in the opposite direction, and the ply twist of one set of pile yarns being substantially less than the ply twist of the other set, and thereafter subjecting said pile yarns to a wetting treatment whereby to partially release the twist of the 5 harder twisted yarns so as to cause the pile tufts formed by these yarns to elongate and rise above the pile tufts formed by the other lesser twisted yarns which are substantially unaffected by the wetting treatment.

10 3. The method of producing embossed or relief designs in pile fabrics, which comprises weaving a plurality of sets of pile yarns, the yarns of each set being composed of staple length fibers and having a different degree of twist, according to a predetermined pattern, to initially provide a pile surface composed of tufts of substantially uniform height, and thereafter subjecting said pile yarns to a wetting treatment at a temperature of approximately ninety degrees Fahrenheit whereby to partially release the twist of the harder twisted yarns so as to cause the pile tufts formed by these yarns to elongate and rise above the pile tufts formed by the other lesser twisted yarns which are substantially unaffected by the wetting treatment.

15 4. The method of producing embossed or relief designs in pile fabrics, which comprises mechanically plying a plurality of individually twisted pile yarns in a direction opposite to the single twist, mechanically plying a second set of pile yarns in the opposite direction to the single twist and in the same direction as but with a lesser twist than the ply twist of the first mentioned plied yarn, weaving said plied yarns according to a predetermined design to initially provide a pile surface composed of tufts of substantially uniform height, and thereafter subjecting said pile yarns to a wetting treatment whereby to partially release the twist of the 20 harder twisted yarns so as to cause the pile tufts formed by these yarns to elongate and rise above the pile tufts formed by the other lesser twisted 25 yarns which are substantially unaffected by the wetting treatment.

30 5. The method of producing embossed or relief designs in pile fabrics, which comprises mechanically plying a plurality of individually twisted pile yarns in a direction opposite to the single twist, mechanically plying a second set of pile yarns in the opposite direction to the single twist and in the same direction as but with a lesser twist than the ply twist of the first mentioned plied yarn, weaving said plied yarns according to a predetermined design to initially provide a pile surface composed of tufts of substantially uniform height shearing said pile tufts to even the same, thereafter subjecting said pile yarns to a wetting treatment whereby to partially release the twist of the harder twisted 35 yarns so as to cause the pile tufts formed by these yarns to elongate and rise above the pile tufts formed by the other lesser twisted 40 yarns which are substantially unaffected by the wetting treatment, drying the fabric, and subsequently shearing the pile tufts forming the high pile areas to even the same.

45 6. The method of producing embossed or relief designs in pile fabrics, which comprises mechanically plying a plurality of individually 50 twisted pile yarns in a direction opposite to the single twist, treating the plied yarn in an aqueous bath having a temperature of approximately 55 120 degrees Fahrenheit to temporarily set the 60 ply twist, mechanically plying a second set of pile 65

- yarns in the opposite direction to the single twist and in the same direction as but with a lesser twist than the ply twist of the first mentioned plied yarn, weaving said plied yarns according to a predetermined design to initially provide a pile surface composed of tufts of substantially uniform height, and thereafter subjecting said pile yarns to a wetting treatment whereby to partially release the twist of the harder twisted 5 yarns so as to cause the pile tufts formed by these yarns to elongate and rise above the pile tufts formed by the other lesser twisted yarns which are substantially unaffected by the wetting treatment.
15. 7. The method of producing embossed or relief designs in pile fabrics, which comprises weaving a plurality of sets of pile yarns, the yarns of each set being composed of staple length fibers and having a different degree of twist, according to a predetermined pattern to initially provide a pile surface composed of tufts of substantially uniform height, and thereafter subjecting said pile yarns to a wetting treatment in solutions of chlorinated lime and formic acid, whereby to 20 partially release the twist of the harder twisted 25 yarns so as to cause the pile tufts formed by these yarns to elongate and rise above the pile tufts formed by the other lesser twisted yarns which are substantially unaffected by the wetting treatment.
8. The method of producing embossed or relief designs in pile fabrics, which comprises weaving a plurality of sets of pile yarns, the yarns of each set having a different degree of twist, and being composed of staple length fibers, to form a surface which is composed of pile tufts initially having substantially uniform height, and thereafter partially releasing the twist of said harder twisted pile yarns in such manner that the tufts formed thereby elongate and thereby form higher pile areas according to a predetermined design, which have distinct contrast with the lower pile areas composed of the other tufts.
40. 9. A pile fabric the surface of which consists

of twisted pile yarns composed of staple length fibers forming tufts of different heights arranged in a predetermined design, the bases of the higher pile tufts being harder twisted than the bases of the lower pile tufts.

10. A pile fabric consisting of twisted pile yarns composed of staple length fibers and having the formation of substantially U-shaped pile tufts, the bases of which are bound in between yarns of a backing fabric, the pile tufts being of different 10 heights according to a predetermined design, and the bases of the higher pile tufts being harder twisted than the bases of the lower pile tufts.

11. A pile fabric as claimed in claim 9, wherein certain of the pile tufts are composed of a greater 15 number of pile yarns plied together than the other pile tufts.

12. A pile fabric as claimed in claim 9, wherein the higher pile tufts are composed of a greater 20 number of pile yarns plied together than the other pile tufts.

13. A pile fabric consisting of a plurality of sets of twisted pile yarns composed of staple length fibers and forming substantially U-shaped pile tufts having their bases bound between the yarns 25 of a backing fabric, the pile tufts being of different heights and arranged in a predetermined design, the bases of the higher pile tufts formed by one set of pile yarns being harder twisted than the bases of the other pile tufts, and at least the 30 free ends of the pile tufts forming the pile surface being substantially spread open and completely concealing the backing fabric.

14. A pile fabric, the pile surface of which is composed of twisted pile yarns composed of staple length fibers and forming tufts of different 35 heights arranged in a predetermined design, the respective pile areas formed by the relatively high and low pile tufts being of substantially uniform density, and the bases of the higher pile tufts 40 being harder twisted than the bases of the lower pile tufts.

HAROLD H. FONDA.